

1

2,756,157

**PREPARATION OF MONOCRYSTALLINE RUTILE**

Malcolm D. Beals, Fanwood, N. J., and James F. Miller, Lancaster, Ohio, assignors to National Lead Company, New York, N. Y., a corporation of New Jersey

No Drawing. Application August 12, 1953,  
Serial No. 373,884

4 Claims. (Cl. 106—42)

The present invention relates to rutile single crystal boules modified with respect to color and certain other physical properties, and to methods for the production of such boules.

Rutile is one of the three known crystal modifications of titanium dioxide. When substantially pure, a massive single crystal of rutile has gem-like properties with a very light straw color and reflectance, refraction and brilliance greater than that of a diamond. By means of the present invention rutile single crystals may be produced which have a nearly water-white color. In addition, the present invention permits finishing the boule by reoxidation in considerably less time than is required for a pure rutile single crystal boule.

The principal object of the present invention is the preparation of rutile single crystal boules having nearly water-white color. Another object of the invention is a method for producing a finished, oxidized rutile single crystal boule in considerably less time than is required for the preparation of a finished oxidized pure rutile single crystal boule. These and other objects of the present invention will become apparent from the following description.

In its broadest aspect the present invention contemplates a rutile single crystal boule containing a small amount of an oxidic compound of gallium in solid solution and characterized by having a nearly water-white color. This water-white single crystal may be prepared according to the method of the present invention by progressively fusing a mixture of finely divided  $TiO_2$  containing a small amount of an oxidic compound of gallium in a flame carrying an excess of an oxidizing gas and thereafter oxidizing boule so formed.

In this description of the present invention the word "boule" is used in its currently accepted meaning to denote a characteristic shape or form of an artificially prepared massive single crystal having a rounded end, or meniscus, a more or less rod-like body portion and a tapering end, giving an overall appearance in profile of an almond, or carrot.

The general method to which the present invention relates is that described in another of assignees' applications, that is in co-pending application Serial No. 286,853, filed May 9, 1952, and now abandoned, for the preparation of pure rutile single crystal boules.

According to the preferred method of the present invention, there is employed as starting material a substantially pure  $TiO_2$  which is very fine, fairly uniform and possesses an open structure with units capable of being rapidly melted. A  $TiO_2$  having an ultimate unit particle size of approximately 0.1 micron has proved especially satisfactory. In general, material having an average particle size above about 5 microns should be avoided because such particles do not satisfactorily fuse under the conditions of the invention. A preferred method for preparing a  $TiO_2$  starting material especially adapted for the production of rutile single crystal boules is described in U. S. Patent No. 2,521,392, issued September 5, 1950,

2

wherein the double salt ammonium-titanium-sulfate is calcined until all of the ammonia and sulfate has been removed by volatilization.

Substantially any oxidic compound of gallium can be added to the feed material, for example, the sesqui-oxide or any oxidic compounds which form the oxide at the temperatures employed in the preparation of the rutile boules.

According to the present invention the small amount of gallium compound may be mixed with the  $TiO_2$  starting material in any convenient manner, for instance, by dry mixing. A more uniform mixture and, therefore, a preferred mixture may be prepared by adding gallium oxide as a powder, slurry, or solution to the double salt, ammonium-titanium-sulfate prior to calcination.

The amount of gallium compound to be added to the  $TiO_2$  starting material should not exceed about 1.0%, calculated as gallium oxide based on the weight of the  $TiO_2$ . The lower limit which is effective is about 0.05%. When the amount of gallium oxide is increased substantially above about 1.0% resulting boules tend to fracture and this is to be avoided. With amounts of gallium oxide of about 1.0% and below a complete solid solution of the gallium oxide in the  $TiO_2$  is formed from which a high quality unfractured boule is produced.

In progressively fusing the starting mixture of  $TiO_2$  and gallium oxide there should be employed a flame which carries an excess of an oxidizing gas, preferably oxygen. Preferably the fusion is carried out according to the method described in application Serial No. 286,853 supra, in which the particles of the starting mixture are entrained in a stream of oxygen in a tube constituting the center of a burner consisting of three concentric tubes. In this burner hydrogen is introduced to the flame through the intermediate tube and additional oxygen in excess over the amount required to combine with the hydrogen is introduced through the outer tube. Preferably, the ratio of oxygen to hydrogen by volume should be about 1:1 and should not be less than about 8.5 parts of oxygen to 9.5 parts hydrogen by volume.

The excess of oxygen in the flame is necessary because at elevated temperatures, titanium dioxide gives up oxygen and is converted to lower, or sub-oxides of titanium, e. g.  $Ti_2O_3$ . This loss of oxygen proceeds with considerable rapidity under conditions produced by an oxy-hydrogen flame wherein the  $TiO_2$  is fused and the loss is accelerated when the flame is neutral or reducing. Under such conditions the formation of lower, or sub-oxides of titanium, is so great that mixtures of small crystals of various oxides of titanium are produced rather than a single crystal boule.

Even when operating with an excess of oxygen the boule as produced has a generally deep blue-black color indicative of some deficiency in oxygen. Therefore, in order to produce the nearly water-white boule of the present invention, the blue-black boule has to be re-oxidized.

The reoxidation of the boule is preferably carried out by heating the blue-black boule in an oxidizing atmosphere, for instance, air or oxygen. The temperature of the treatment should be within the range from about 650° C. to about 1500° C. It has been found that temperatures to any extent below 650° C. oxygen will not be appreciably incorporated into the rutile single crystal while temperatures above 1500° C. are expensive and difficult to maintain. The heating should be continued until the boule obtains the maximum degree of lightness of color, this time will usually be about one-quarter of that required to fully oxidize a pure rutile boule.

As produced, the gallium oxide containing rutile boule has a more or less frosted outer surface. When split, the interior surfaces of the pieces are vitreous and shiny and nearly water-white. They may be cut and polished to form beautiful gems, more brilliant than diamonds and

## 3

having a white color compared to the characteristic straw or light yellow color of pure rutile.

The foregoing description has been given for purposes of illustration, but the invention is not to be limited thereto and various modifications and variations within the scope of the appended claims may be employed.

We claim:

1. A single crystal of synthetic rutile consisting essentially of titania and from about 0.05% to about 1.0% of an oxidic compound of gallium.

2. A single crystal of synthetic rutile consisting essentially of titania and from about 0.05% to about 1.0% gallium oxide.

## 4

3. A method for synthesizing a substantially water-white single crystal of rutile consisting of fusing a powder containing titania and from about 0.05% to about 1.0% of an oxidic compound of gallium, crystallizing the fused material and heating the crystallized material in an oxidizing atmosphere of oxidizing gas until the water-white color is obtained.

4. The method according to claim 3 in which the crystallized material is heated in an atmosphere of oxygen at a temperature between about 650° C. and 1500° C.

No references cited.